

# United States Patent

[11] 3,620,720

[72] Inventors **Philippe Galmiche**  
Clamart;  
**Andre R. Hivert, Pontoise; Michel E.**  
**Marty, Paris, all of France**  
709,794  
[21] Appl. No.  
[22] Filed Mar. 1, 1968  
[45] Patented Nov. 16, 1971  
[73] Assignee Office National D'Etudes Et De Recherches  
Aerospatiales (par abreviation:  
O.N.E.R.A.)  
Chatillon-sous-Bagneux, France

[54] **PROCESS FOR PRODUCING METALLIC**  
**MATERIALS CONTAINING THORIA**  
8 Claims, No Drawings

[52] U.S. Cl. .... **75/206,**  
23/345, 29/182.5, 75/211, 252/301.1, 264/5  
[51] Int. Cl. .... **C22c 39/50**  
[50] Field of Search .... 252/301.1;  
264/5; 23/345; 29/182.5; 75/211, 206

| [56] References Cited |         |                 |
|-----------------------|---------|-----------------|
| UNITED STATES PATENTS |         |                 |
| 2,099,325             | 6/1933  | Zellman .....   |
| 3,143,789             | 8/1964  | Iller .....     |
| 3,159,908             | 12/1964 | Anders .....    |
| 3,278,281             | 10/1966 | Ehringer .....  |
| 3,285,736             | 11/1966 | Brinn .....     |
| 3,310,400             | 3/1967  | Alexander ..... |
| 3,422,167             | 1/1969  | Bowman .....    |
| 3,489,553             | 1/1970  | Duletsky .....  |

## FOREIGN PATENTS

|           |        |               |
|-----------|--------|---------------|
| 1,232,353 | 1/1967 | Germany ..... |
| 39/5913   | 6/1962 | Japan .....   |

Primary Examiner—Carl D. Quarforth

Assistant Examiner—Arthur J. Steiner

Attorneys—Sylvester J. Liddy, John J. Hart, Joe E. Daniels  
and Dayton R. Stemple

**ABSTRACT:** The thoria used for the dispersion is obtained by pyrolysis of a chelated compound of thorium whose anion comes from a diketone  $\beta$ , this compound being preferably thorium acetylacetoneate.

**PROCESS FOR PRODUCING METALLIC MATERIALS  
CONTAINING THORIA**

The present invention relates, on the one hand, to metallic materials comprising essentially a metallic mass (pure metal or alloy), called in terms of the art matrix, in the midst of which are incorporated, in the form of a dispersed phase, fine particles of thoria ( $\text{ThO}_2$ ) whose presence improves the characteristics of the matrix, notably from the point of view of its resistance to plastic deformation at high temperatures and from the point of view of its resistance to oxidation, and on the other hand, to processes for producing such metallic materials containing a dispersed phase of thoria. The invention is more particularly, but not exclusively, concerned with metallic materials of the type in question and processes for their production, in which the matrix in which the thoria is incorporated is a refractory material (metal or alloy), and, in particular, a refractory material whose base consists of nickel and/or cobalt and/or iron; in addition, this matrix can possibly contain addition elements such as, in particular, chromium, zirconium, aluminum, titanium, tungsten, molybdenum, etc.

Before dealing with the principal feature of the invention, it is appropriate to mention that, in the past, the thoria incorporated in the materials of the type in question was obtained by pyrolysis of certain compounds of thorium (oxalates, nitrates, carbonates, hydroxides, etc...) which, even after a pyrolysis pushed up to high temperatures (of the order of 1,000° C.), give a thoria accompanied by residues difficult to eliminate due to the fact that they are chemically bonded. In other words, by starting from these compounds of thorium, it was impossible to obtain, in simple and economical conditions, fine thoria sufficiently pure, the presence of chemically bonded residues compromising the high-temperature behavior of the metallic material containing a dispersed phase of impure thoria.

The chief object of the invention is to provide materials and processes of the type in question that fulfill the various considerations of practice, and in particular, that no longer have the disadvantages, mentioned above, of the known materials and processes of the same type which use, for the production of the thoria for the dispersed phase, thorium compounds giving an impure thoria, that is to say accompanied by residues altering the high-temperature behavior of the metallic material finally obtained containing the dispersed phase of thoria.

The invention consists, principally, in adopting, as the thoria which is to form the dispersed phase in the materials of the type in question, thoria obtained by pyrolysis of a chelated compound of thorium whose anion comes from a diketone  $\beta$ , this compound being preferably thorium acetylacetoneate, such a thoria being practically stoichiometric, that is to say exempt of residues detrimental to the high-temperature behavior of the finally obtained metallic material containing the dispersed phase of thoria.

Apart from this principal feature, the invention comprises certain other features which are preferably used at the same time, and which will be more explicitly described hereafter.

Preferred embodiments of the invention will now be described, merely by way of example. In these examples, the metallic material in question is a refractory metallic material having a matrix whose base is nickel and/or cobalt in which the thoria is dispersed in a homogeneous manner, the thoria being in an appropriately divided state (particles of granulation at the most of the order of 0.1 microns.)

In accordance with the principal feature of the invention, one uses, as the thoria which is to form the dispersed phase in the above-mentioned matrix, thoria obtained by pyrolysis, at a temperature higher than 550° C. and preferably lower than 900° C., of a chelated compound of thorium whose anion comes from a diketone  $\beta$ .

The thoria thus obtained has the advantage of being stoichiometric, that is to say exempt of any residue, and particularly of water of crystallization or of OH groups, which is not the case with the thoria obtained from other oxygenated compounds of thorium such as: oxalate, nitrate, hydrocarbonate, hydroxide, etc...

Now, experience has shown that, if the thoria dispersed in a metallic matrix containing nickel and/or cobalt is a thoria accompanied by residues (in particular water of crystallization), the high-temperature behavior of this matrix is seriously compromised due to the fact that an uncontrolled dispersion of these residues takes place in the midst of the matrix; such a disadvantage is particularly serious when the metal material containing nickel and/or cobalt and a dispersed phase of thoria is intended for the manufacture of pieces to be exposed to high temperatures such as, in particular, blades, fixed or movable, of gas turbines.

The use, for the formation of a dispersed phase, of stoichiometric thoria obtained by pyrolysis of a chelated compound of thorium whose anion comes from a diketone  $\beta$  avoids precisely the disadvantage, mentioned above, of refractory materials having nickel and/or cobalt containing a dispersed phase of a thoria obtained from thorium salts other than a chelated compound of the type indicated.

The purity of the thoria obtained from such a chelated compound of thorium can be explained, to a certain degree, by the fact that the chelated compounds in question, which are strong chelates, have only a small propensity to form compounds of addition, and in particular, crystallize easily in the anhydrous state.

Among other chelated compounds of thorium whose anion comes from a diketone  $\beta$ , which chelated compounds can be used for the production of a pure thoria, can be cited, in particular, thorium benzoylacetonate and thorium dibenzoylmethanate, and above all, thorium acetylacetoneate which appears to be the most advantageous of the chelated compounds in question for the present purpose, that is to say for obtaining, in a final material having a dispersed phase of thoria, a pure and fine thoria in simple and economical conditions.

It seems appropriate, at this point of the description, to mention that the production of pieces formed of a refractory metallic material having a dispersed phase of thoria conforming to the invention falls within the scope of conventional metallurgy of powders, that is to say of processes according to which an initial mixture of powders is first of all subjected to a forming treatment, then to a sintering treatment.

Various embodiments of the invention will now be examined, which permit such an initial mixture of powders to be obtained (to which mixture a treatment of the metallurgy of powders will then be applied) in the most interesting case in which the matrix of the refractory material has a base of nickel and/or cobalt (i.e. the base consists of these two metals or of only one of these metals) and in which the thoria dispersed in this refractory material is pure and fine thoria obtained by pyrolysis of thorium acetylacetoneate, this initial mixture of powders being able, in the case envisaged, to contain nickel and/or cobalt and such a pure and fine thoria, as well as possibly complementary constituents (other than nickel and/or cobalt) of the matrix.

For the purpose of simplifying the description, and also because it is a practically envisageable application of the invention, and hence can serve as an example, it will be supposed, in the following, that the matrix in which the pure and fine thoria is to be dispersed is constituted exclusively of nickel and/or cobalt, the initial mixture of powders which has just been mentioned them being an intimate mixture of powders of nickel and/or cobalt (these metals being either codiffused or not) and of thoria.

According to the first embodiment, in a first operational stage, the pure and fine thoria can be prepared by pyrolysis of thorium acetylacetoneate at a temperature higher than 550° C. and preferably lower than 900° C. (this temperature being advantageously in the neighborhood of 700° C.); then an intimate mixture can be mechanically prepared of the pure and fine thoria thus obtained with some powder of nickel and/or cobalt of fine granulation (grains of average dimension smaller than 10 microns and preferably of the order of 2 to 5 microns), this embodiment basically amounting to putting in presence and to mixing intimately in a mechanical manner two

solid phases formed respectively by the powder of pure and fine thoria and the powder of nickel and/or cobalt.

A quantitative example according to this first embodiment will now be given.

**EXAMPLE I (matrix formed of nickel)**

a. Preparation of the thorium acetylacetoneate.

Fifty grams of thorium nitrate,  $\text{Th}(\text{NO}_3)_4 \cdot 6\text{H}_2\text{O}$ , are dissolved in one litre of water.

Ammonia liquor is added until a pH of the order of 10 is obtained, which has the effect of making the thorium hydrate precipitate.

This thorium hydrate is washed and filtered on a very fine fabric, after which a final washing is carried out with ethyl alcohol.

The last traces of water are eliminated by means of ternary alcohol-benzine-water azeotrope by addition to the filtrate of one litre of ethyl alcohol at 95 percent and of 600 cm.<sup>3</sup> of benzine, after which the product is dried at 60° C. until three-fourths of the solution has evaporated.

Acetylacetone is added until complete dissolution is reached.

The product is dried, which has for its effect to crystallize the thorium acetylacetoneate  $\text{Th}(\text{C}_5\text{H}_7\text{O}_2)_4$  which is then ground in a mortar so as to obtain a powder whose color is yellow.

b. Pyrolysis of the thorium acetylacetoneate.

The thorium acetylacetoneate thus obtained is placed in a nickel container and heated in an oven at 600° C. for a duration of about one-half hour, this treatment having the effect of causing the fusion of the thorium acetylacetoneate which then blisters to give finally a pure and very friable thoria foam.

c. Mechanical incorporation of the thoria in the nickel powder.

In a ball mill comprising a nickel vat of about 4 litres half full of nickel balls of about 12 millimeters in diameter, there are introduced 2 kilograms of very pure and very fine nickel powder coming from the pyrolysis of nickel carbonyl (granulation of from 2 to 5 microns), 60 grams of thoria obtained as indicated above under (b) and 850 cm.<sup>3</sup> of benzine.

The grinding is continued for 24 hours and the product is then centrifuged, dried in a drying oven at 80° C. and calcined in hydrogen at 850° C. for one hour.

An intimate mixture of powders of nickel and of pure and fine thoria is thus obtained, and this mixture will then be subjected to a treatment of metallurgy of powders to produce refractory pieces of nickel containing a dispersed phase of thoria, which are the pieces originally intended to be produced.

It is appropriate to mention that the process described with respect to this Example I is entirely applicable in the case in which the matrix is constituted of cobalt or of a nickel-cobalt alloy.

Although one can hope to obtain satisfactory pieces by this embodiment, it must nevertheless be admitted that it is difficult to obtain, merely by mechanical means, an intimate mixture with homogeneous dispersion of two solid phases having very fine granulation, and there is a risk that the dispersion of the thoria will not have a maximum homogeneity.

Thus, it seems preferable to use one of the two embodiments which will now be described, and which have this common characteristic of bringing into play at least one liquid phase for the preparation of the mixture of powders, and of forming the pure and fine thoria in situ, that is to say in the presence of the powder of powder of nickel and/or cobalt or of a compound of nickel and/or of cobalt from which such a powder of nickel and/or cobalt can be obtained; these two embodiments have the considerable advantage, due to the fact that they bring into play at least one liquid phase, of avoiding the constraints inherent in the first embodiment and of consequently assuring an absolutely homogeneous dispersion of the thoria.

Thus according to the second embodiment of the invention, a liquid phase (containing the thorium) is put in the presence

of solid phase (containing the metal — in the present case, nickel and/or cobalt). To do this, advantageously, a solution of thorium acetylacetoneate is used to wet a fine powder of nickel and/or cobalt or a compound of nickel and/or cobalt adapted to give a nickel oxide and/or a cobalt oxide reducible by pyrolysis effected in the relatively low temperature zone suitable for the formation of pure and fine thoria by pyrolysis of thorium acetylacetoneate.

As solvent for the thorium acetylacetoneate, one can use, in particular, ethanol, acetone, ether, and better still, acetylacetone.

The wetting thus achieved permits an intimate mixture of the constituents to be obtained, and the pyrolysis effected afterwards at a temperature comprised between 550° C. and 900° C. has the effect of transforming the thorium acetylacetoneate into pure and fine thoria, and when the starting product is a powder of a compound of nickel and/or cobalt, of transforming this compound directly into metal (the case in which the starting products are oxalates for example) or again into oxides reducible in hydrogen (the case in which the starting products are carbonates for example).

A quantitative example of this second embodiment of the invention will now be given.

**EXAMPLE II**

Three kilograms of oxalate of nickel and/or cobalt are introduced into a mixer provided with a heating device (for example a "WERNER" mixer), and there is incorporated by rotation into this cold oxalate, 64 grams of thorium acetylacetoneate dissolved in 900 cm.<sup>3</sup> of acetylacetone.

The cold mixing is continued for one hour, then the temperature is progressively raised to 130° C., which causes the volatilization of the solvent by ceaselessly renewing the surface contacts.

The dry powder thus obtained is placed in a nickel container and introduced into an adjustable temperature oven capable of bringing this powder to a temperature of the order of 500° C. in 4 hours in ordinary atmosphere, after which this temperature is maintained for 1 hour. After cooling, the powder is placed in a nickel cup and the pyrolysis is carried out in dry hydrogen at 700° C for 2 hours.

An intimate mixture is thus obtained of powders of nickel and/or cobalt and of pure and fine thoria dispersed in a homogeneous manner, this mixture being suitable as the initial mixture for a subsequent treatment of the metallurgy of powders.

Finally, according to a third embodiment, two liquid phases are put in the presence of one another, these two liquid phases containing respectively the thorium and the metal (in this case, nickel and/or cobalt); to do this, advantageously, thorium acetylacetoneate in the melted state is mixed with some acetylacetoneate of the metal or of the metals also in the melted state, these two compounds being miscible in all proportions.

Then a simultaneous pyrolysis is carried out of the two compounds thus mixed, which leads to a pure and fine thoria excellently dispersed in the powder of nickel and/or cobalt.

To finish, a quantitative example of this third embodiment will now be given.

**EXAMPLE III**

a. Preparation of the acetylacetoneate of nickel and/or of cobalt.

One hundred grams of nitrate of nickel and/or of cobalt are dissolved in 500 cm.<sup>3</sup> of water, and a solution of 50 grams of ammonium carbonate in 500 cm.<sup>3</sup> of water is added.

A precipitate of carbonate of nickel and/or of cobalt is thus obtained which is washed, centrifuged and dried, then incorporated progressively into 200 cm.<sup>3</sup> of boiling acetylacetone, which permits, after evaporation of the excess acetylacetone, crystals of metallic acetylacetoneate of nickel and/or of cobalt, or again mixed crystals of acetylacetoneate of nickel and of cobalt, to be obtained.

b. Mixture of the acetylacetoneates of nickel and/or of cobalt and of thorium.

A mixture formed by one kilogram of acetylacetoneate of nickel and/or of cobalt, 17 grams of thorium acetylacetoneate and 750 cm.<sup>3</sup> of acetylacetone are heated to ebullition.

When the solution becomes very viscous, it is placed in a vacuum dryer where the evaporation is continued at 150° C. A foam is thus obtained which is then treated like the dry powder of Example II.

In any case, and whatever embodiment is adopted, an initial mixture of powders is provided which has, for the production of refractory pieces having a base of nickel and/or of cobalt containing a dispersed phase of thoria, the advantages (explained previously) inherent in the purity and the fineness of the thoria used, and the initial mixture of powders in question lends itself to all the conventional operations of the metallurgy of powders (forming, sintering, sheathing, hot drawing, cold working, etc....).

Moreover, in the case of the second and third embodiments, an excellent dispersion of the pure and fine thoria is assured in the constituent of constituents of the matrix, due to the fact that this thoria is formed in situ and by a process (forming an essential part of the invention) bringing into play compounds of thorium whose pyrolysis is achieved at relatively low temperatures (of the order of 550° C. for thorium acetylacetoneate); this permits pollution to be avoided of the metallic phase and corrélatively of the thoria by reaction with that polluted metallic phase, which is very advantageous, since any pollution would be disastrous for the refractory metallic product containing the dispersed phase of thoria.

Although the present invention has been described with particular reference to particular embodiments, it should be understood that the invention should not be limited thereto, as there might be various modifications made without departing from the scope or spirit of this invention.

What we claim is:

1. In a process of producing a sintered metallic material having as its base at least one metal powder and containing a dispersion of thoria, the steps of, supplying a chelated com-

pound of thoria whose anion comes from a  $\beta$  diketone, pyrolyzing said chelated compound of thorium to prepare said thoria, intimately mixing said thoria with at least one said metal powder forming the base of said metallic material, and subsequently processing the mixture by powder metallurgy.

2. A process according to claim 1 which comprises intimately mixing a liquid phase containing said chelated compound of thorium with a solid phase containing at least one said metal, and pyrolyzing said mixture.

10 3. A process according to claim 1 which comprises intimately mixing a first liquid phase containing said chelated compound of thorium with a second liquid phase containing at least one said metal, and pyrolyzing said mixture.

15 4. A process according to claim 1 wherein said chelated compound of thorium is thorium acetylacetoneate, and said pyrolysis if effected at a temperature in the range 550° C. to 900° C.

5. A process according to claim 4 wherein said thorium acetylacetoneate is pyrolyzed at a temperature in the neighborhood of 700° C. to form a foam of thoria in the solid state, and said solid state thoria is intimately mixed by grinding with a powder containing at least one said metal chosen from the class consisting of nickel and cobalt.

20 6. A process according to claim 2 wherein said liquid phase is a solution of thorium acetylacetoneate in an appropriate solvent, and said solid phase is a powder containing at least one said metal chosen from the class consisting of nickel and cobalt.

7. A process according to claim 6 wherein said solvent is acetylacetone, and said pyrolysis is effected at a temperature in the range 500° C. to 900° C.

30 8. A process according to claim 3 wherein said first liquid phase comprises thorium acetylacetoneate and said second liquid phase comprises an acetylacetoneate of at least one said metal chosen from the class consisting of nickel and cobalt.

\* \* \* \* \*

40

45

50

55

60

65

70

75